

1

3,671,242

### SILVER SALT DIFFUSION PROCESS

Werner Liebe, Siegfried Petersen, and Anita von Konig, Leverkusen, Germany, assignors to Agfa-Gevaert Aktiengesellschaft, Leverkusen, Germany  
No Drawing. Filed Dec. 30, 1969, Ser. No. 889,352  
Claims priority, application Germany, Jan. 25, 1969,  
D 19 03 741.3

U.S. Cl. 96—29

Int. Cl. G03c 5/54

2 Claims

### ABSTRACT OF THE DISCLOSURE

The image tone of silver images produced by the silver salt diffusion process is unproved by performing the development in the presence of 1,2,4-triazine blue toners.

The invention relates to an improvement in the silver salt diffusion process in which the exposed silver halide emulsion layer is developed in the presence of 1,2,4-triazines as blue toners.

It is already known that the production of an image in the reception layer is advantageously accomplished in the presence of components which influence the color of the silver precipitated in the reception layer. Such compounds form silver salts difficultly-soluble in water and in the sodium thiosulfate solution. Some efficacy is, for example, shown by the compounds described in German Pat. No. 473,000 and 890,755.

These compounds have, however, several disadvantages. In particular they retard the formation of the positive image in the silver salt diffusion process, so that longer contact times are necessary. It is, however, desirable to reduce the necessary copying times, and so need exists for compounds which accelerate the diffusion process and the image formation in the positive material and simultaneously produce, as far as possible, a deep black silver image.

Although the mercapto triazoles described in U.S.-specification 3,307,944 satisfy the practical requirements as regards their blue toner effect and, furthermore, do not retard the diffusion of silver halide, they are unsatisfactory in cases where several positive copies are to be produced from one exposed negative. In such cases it is found that in the presence of these mercapto triazoles the second copy has insufficient covering.

It is among the objects of the invention to improve the silver salt diffusion process so that several positive copies of higher density and with a neutral black image tone can be obtained from one exposed negative.

We now have found a silver salt diffusion process comprising the steps of exposing a supported silver halide emulsion layer, developing the exposed layer in the presence of solvents for the silver halide and in contact with a reception sheet containing development nuclei for the transferred silver halide, wherein the development is performed in the presence of 1,2,4-triazine blue-toners of the following formula:



2

or its tautomeric forms



wherein represents:

R<sub>1</sub>=hydrogen, alkyl containing up to 3 carbon atoms, alkoxy carbonyl, acyl in particular acyl derived from lower aliphatic carboxylic acids having up to 5 carbon atoms, such as acetyl or carbamoyl, the amide group of which may be substituted, preferably with short chain alkyl radicals containing up to 3 carbon atoms or an aryl group, preferably a phenyl group, and R<sub>2</sub>=hydrogen or alkoxy carbonyl containing up to 5 carbon atoms, at least one of the two R<sub>2</sub> groups being hydrogen.

The following are examples of compounds which have proved to be suitable

1.

25



2.

35



3.

40



4.

45



5.

50



6.

55



The 1,2,4-triazine toners may be prepared by known processes, for example by those described in German patent specification (P 1 670 979.8).

65 The compounds are preferably added in quantities of 1 to 200 mg. per m.<sup>2</sup> of image receiving layer and/or similar quantities per liter of developer. Most of the

## 3

compounds are easily soluble in aqueous alkaline solution and can therefore be added to the known developers for the silver salt diffusion process without the need for changing the formulation of the developer. As additives for the alkaline developer solution are preferred 1,2,4-triazines with free mercapto group since these compounds are stable in caustic potash solution. Their activity is only slightly affected by the development temperature but development is preferably carried out at temperatures of between 15 and 35° C.

## EXAMPLE 1

## Preparation of the reception layer

A baryta coating is applied to a support of paper (80 g. per m.<sup>2</sup>) using the following solution:

6 g. of a 50% aqueous slurry of barium sulfate  
20 ml. of a 10% aqueous gelatin solution  
8 ml. of a 50% aqueous emulsion of polyvinyl acetate water up to 100 ml.

The baryta layer is dried and then coated with a nucleated layer using the following casting solution:

4.5 g. of propylene glycol alginate  
12.5 mg. of silver sulfide in the form of an aqueous colloidal solution  
20 ml. of a 50% aqueous gelatin solution  
1.5 ml. of a 30% aqueous solution of potassium bromide  
1.2 ml. of a 30% aqueous solution of saponin  
7.5 g. of sodium thiosulfate made up with water to 300 ml.

Four portions of the above composition are prepared and a certain quantity of one of the 1,2,4-triazine blue toners is added to each of these portions before casting.

- Sample 1: Addition of 0.1 g. of compound 1.  
Sample 2: Addition of 0.05 g. of compound 2.  
Sample 3: Addition of 0.02 g. of compound 5.  
Sample 4: Addition of 0.15 g. of compound 6.

The layer is applied in such a thickness that it contains approximately 1.1 g. of sodium thiosulfate per m.<sup>2</sup>.

Another layer of the following casting solution is applied to the layer described above:

3.5 g. of sodium alginate  
10 g. of sodium thiosulfate  
0.8 ml. of a 30% aqueous potassium bromide solution  
8 ml. of a 30% aqueous saponin solution made up with water to 350 ml.

This layer is applied in such thickness that it contains about 0.6 g. of sodium thiosulfate per m.<sup>2</sup>.

## Processing

The above reception layer is brought into contact with an exposed silver chloride emulsion layer and developed in the following developer bath in a conventional processing apparatus:

|                          | G.  |
|--------------------------|-----|
| Sodium sulfite anhydrous | 60  |
| Hydroquinone             | 14  |
| 1-phenyl-3-pyrazolidone  | 1.2 |
| Sodium hydroxide         | 11  |
| Potassium bromide        | 2   |
| Water up to 1 l.         |     |

After production of the first copy, the process is repeated so that a second copy is also obtained.

The copies obtained have an excellent neutral black image tone after the usual contact times of about 5 to 10 seconds. The second copy is also in all cases of good quality.

If the process is carried out in the same way but using a mercapto triazole blue toner described in U.S. Pat. No. 3,307,944 in the reception layer instead of the 1,2,4-tri-

## 4

azines according to the invention, a first copy of excellent quality is obtained but the second copy has insufficient covering.

## EXAMPLE 2

5 An exposed silver chloride emulsion layer on a paper support is brought into contact with the reception layer described in Example 1 with the exception that the reception layer does not contain any blue toner.

Development is carried out with the following bath in a conventional processing apparatus:

|                           | G.   |
|---------------------------|------|
| Sodium sulfite            | 75   |
| Hydroquinone              | 15   |
| 1-phenyl-3-pyrazolidone   | 1.2  |
| Sodium hydroxide          | 12   |
| 1,2,4-triazine blue toner | 0.04 |

The following compounds are tested:

20 Sample 1: Addition of Compound 5 to the developer.  
Sample 2: Addition of Compound 1 to the developer.

Using a contact time of 5 to 10 seconds, first and second copies with good neutral black tones are obtained. Without the addition of blue toner to the developer, the copies are brown in color. When using a blue toner of 25 the type described in U.S. Pat. No. 3,307,944 the second copy is unsatisfactory in quality.

What is claimed is:

30 1. In a silver salt diffusion process for producing a plurality of copies from an exposed silver halide emulsion comprising the steps of exposing a supported silver halide emulsion layer and developing the exposed layer in the presence of a silver halide solvent while in contact with a reception layer containing development nuclei for silver halide, the improvement consisting of developing in effective contact with a 1,2,4-triazine blue toner of the following formulae:



35 45 wherein represents:

R<sub>1</sub>=hydrogen, alkyl with up to 3 carbon atoms, alkoxy-carbonyl, acyl or carbamyl, the amide group of which may be substituted by short chain alkyl radicals having up to 3 carbon atoms or aryl, and

50 R<sub>2</sub>=hydrogen or alkoxy-carbonyl with up to 5 carbon atoms, at least one of the R groups representing a hydrogen atom said toner effective in providing a second copy of said exposed layer having coverage equivalent to the first copy.

55 2. The process of claim 1, wherein the blue toner has the following formula:



## References Cited

## UNITED STATES PATENTS

65 3,307,944 3/1967 Weyde et al. ----- 96-66  
3,431,108 3/1969 Willems et al. ----- 96-52

NORMAN G. TORCHIN, Primary Examiner

J. L. GOODROW, Assistant Examiner

U.S. CL. X.R.

96-58

UNITED STATES PATENT OFFICE  
CERTIFICATE OF CORRECTION

Patent No. 3,671,242

Dated June 20, 1972

Inventor(s) Werner Liebe et al

It is certified that error appears in the above-identified patent and that said Letters Patent are hereby corrected as shown below:

Column 2, compound number 3, should read as follows:



Column 4, claim 1, formula 3 should read as follows:



Column 4, claim 2, the formula should read as follows:



Signed and sealed this 29th day of May 1973.

(SEAL)  
Attest;

EDWARD M. FLETCHER, JR.  
Attesting Officer

ROBERT GOTTSCHALK  
Commissioner of Patents